# EUROPEAN PATENT SPECIFICATION

(11) **EP 0 540 557 B1**
(45) Date of publication and mention of the grant of the patent: **16.10.1996**
(21) Application number: 91912843.9
(22) Date of filing: 08.07.1991
(51) Int. Cl.: C11D 3/16, C11D 3/37, C11D 3/00, D06M 15/65

(54) **LIQUID FABRIC SOFTENERS CONTAINING MICROEMULSIFIED AMINO SILANES**
FLÜSSIGE WEICHEMACHER FÜR GEWEBE MIT MIKROEMULGIERTEN AMINOSILANEN
ASSOUPLISSANT LIQUIDE POUR TISSUS CONTENANT DES AMINO SILANES MICROEMULSIFIES

(30) Priority: 23.07.1990 US 557438
(43) Date of publication of application: 12.05.1993
(73) Proprietor: THE PROCTER & GAMBLE COMPANY, Cincinnati, Ohio 45202 (US)
(72) Inventor: COFFINDAFFER, Timothy, Woodrow, Loveland, OH 45140 (US); BUZZEE, Sheila, Gay, Fort Mitchell, KY 41017 (US)
(74) Representative: Canonici, Jean-Jacques
(86) International application number: US9104729
(87) International publication number: WO9201773

(56) References cited:
- EP-A- 0 075 990
- EP-A- 0 138 192
- EP-A- 0 150 872
- EP-A- 0 300 525
- EP-A- 0 417 047
- FR-A- 2 318 268
- US-A- 4 661 577

## Description

### FIELD OF THE INVENTION

This invention relates to fabric care compositions and to a method for treating fabrics in order to improve various properties of the fabric, in particular, reduction of fiber-fiber and yarn-yarn friction.

### BACKGROUND OF THE INVENTION

The use of silicones for softening fabrics, i.e., providing lubrication between fibers and yarns so they move over one another more easily, has been well known for quite some time. In addition, the use of organomodified silicones for textile treatments has also been well documented over the years (See U.S. Pat. Nos.: 4,620,878, Gee, issued Nov. 4, 1986; 4,705,704, Lane et al., issued Nov. 10, 1987; 4,800,026, Coffindaffer et al., issued Jan. 24, 1989; 4,824,877, Glover et al., issued April 25, 1989; and 4,824,890, Glover et al., issued April 25, 1989; also of interest is Brit. Pat. Appln. 87-29,489, Walbeoff, published Dec. 18, 1987). Silicones of this type are typically delivered to textiles in the form of an aqueous emulsion. More recently, much work has concentrated on the aqueous delivery of these systems via microemulsions. The above art suggests that microemulsions have two advantages over conventional "macro" emulsions: (1) they are more stable and (2) they require less mechanical energy to make.

EP-A-0,417,047, published on 13.03.91, discloses a stabilised microemulsion comprising an amine functional silicone together with an ampholytic surfactant, wherein the pH of said microemulsion is less than 7.

EP-A-0,138,192 discloses stabilised microemulsions of amino functional silicone with an insoluble surfactant. Particularly exemplified is a microemulsion containing an aminofunctional silicone and a quaternary ammonium compound in amount of 1.4%.

While hand evaluation of fabrics to determine softness is still practiced widely, about 20 years ago Dr. Sueo Kawabata et al. began evaluating textiles via a mechanical approach. They designed instruments to measure low deformation forces, typical of hand analysis, on fabrics. Although these instruments (commonly known as the Kawabata Evaluation System or KES) were designed to be quality control tools for fabric acceptance, the instruments have also been used to study the effect of fabric treatments. Two such studies have been published by Union Carbide Co.: Sabia, A.J. and Pagluighi, A.M., Textile Chemist and Colorist, Vol. 19, No. 3, March 1987, p. 5; and Barndt, H.J., Sabia, A.J. and Pagluighi, A.M., Textile Chemist and Colorist, Vol. 21, No. 12,, December 1989, p. 16. The shearing instrument, in particular the shearing hysteresis measurement, is believed to be indicative of the ease with which fibers and/or yarns move over one another. Thus, the lower the shear hysteresis value, the better the lubricant.

The term "reduced fiber-fiber/yarn-yarn friction" (reduced friction between individual fibers within the yarn as well as between the yarn strands) as used herein means that the fabric exhibits a lower shear hysteresis value as measured by the KES shearing instrument. While not wishing to be bound by theory, it is believed that a reduction in reduced fiber-fiber/yarn-yarn friction provides better drape, hand, and wrinkle removal during tumble drying and ironing processes due to the fibers being more easily moved over one another.

### SUMMARY OF THE INVENTION

This invention relates to fabric care compositions comprising a microemulsified amine functional silicone agent and a fabric softener for use in a fabric care operation whereby an effective amount of said microemulsified amine functional silicone is deposited on said fabric for reduced fiber-fiber/yarn-yarn friction.

### DETAILED DESCRIPTION OF THE INVENTION

This invention relates to microemulsified amine functional silicone compositions as in the appended claim 1 for reduced fiber-fiber/yarn-yarn friction. In another respect this invention relates to methods of using such microemulsified amine functional silicone compositions in the care of fabrics for reduced fiber-fiber/yarn-yarn friction. Preferred compositions are aqueous fabric softeners. Such compositions are usually added to either the wash or rinse water of a laundering operation. These preferred compositions are aqueous based, water-dispersible compositions which contain from 0.05% to 25%, more preferably from 0.1% to 15% of the microemulsified amine functional silicones. The compositions are diluted in the wash or rinse.

Surprisingly, the Microemulsified Amine Functional Silicones (MAFS) incorporated into a liquid fabric softener composition of the invention exhibit a synergistic behavior when compared to the corresponding "macro" emulsified material. Said differently, used by itself, the MAFS performance for reduced fiber-fiber/yarn-yarn friction is not as good as that of the macroemulsified system; however, in the context of a liquid fabric softener composition of the invention the MAFS composition provides a greater reduction in shear hysteresis values than the corresponding macroemulsion in an analogous liquid fabric softener composition.

A preferred embodiment comprises: a liquid rinse water composition comprising the microemulsified amine functional silicone plus quaternary ammonium fabric softener.

In a preferred execution, 0.1% to 10% by weight of microemulsified amine functional silicone is mixed into a suitable prior art laundry liquid fabric softener composition. The result is a fabric care composition that provides a reduced fiber-fiber/yarn-yarn friction benefit to the treated fabric.

### Silicone Microemulsions

Over the last 5 years, there have been many patents published in the area of silicone microemulsions (U.S. Pat. Nos.: 4,620,878; 4,705,704; 4,824,877; 4,824,890, all supra; also of interest is Brit. Pat. 87-29,489, supra). In this literature, silicone microemulsions have been described as translucent silicone emulsions with average particle sizes smaller than 0.14 microns. In this art, microemulsions are taught as having two advantages over conventional "macro" emulsions: (1) they are more stable and (2) they require less mechanical energy to make. There is no disclosure either that microemulsions can reduce fiber to fiber and/or yarn to yarn friction as compared to macroemulsions when used with a fabric softener. Since microemulsions are inferior in performance to macroemulsions when used alone, any investigation which starts logically with the individual dispersions would discourage further investigation.

The amine functional silicones herein have an average molecular weight of from 1,000 to 100,000, preferably from 1,000 to 50,000, more preferably from 1,500 to 20,000, and can be prepared by emulsion polymerization of low molecular weight polymers and/or monomers, more preferably low molecular weight polymers. Emulsion polymerization can provide a high concentration of microemulsified silicone.

### Some Preferred Embodiments

The preferred composition of this invention is an aqueous dispersion comprising: a microemulsified amine functional silicone wherein the weight ratio of microemulsified amine functional silicone to fabric softener is from 17:1 to 1:350, preferably from 10:1 to 1:100. Even more preferred weight ratios of microemulsified amine functional silicone to fabric softener are from 1:1 to 1:10, and more preferably, from 1:5 to 1:10. These compositions are added to the rinse water for reduced fiber-fiber/yarn-yarn friction and fabric softening benefits.

Suitable fabric softener(s) are selected from the group consisting of:
i. quaternary ammonium compound;
ii. fatty amine compound;
iii. fatty amide compound;
iv. fatty acids;
v. fatty alcohols; and
vi. mixtures thereof.

In the liquid rinse-added compositions of this invention the amount of fabric softener ranges from 2% to 35%, preferably from 4% to 27%, by weight of the total composition. The lower limits are amounts needed to contribute effective fabric softening performance when added to laundry rinse baths in the manner which is customary in home laundry practice. The higher limits are suitable for more concentrated liquid products which require either smaller volume usage or dilution prior to use.

The preferred levels of microemulsified amine functional silicone in such composition can range from 0.05% to 40%; preferably from 0.1% to 20%; and more preferably from 0.5% to 10% by weight of the concentrate.

Suitable fabric softener compounds include quaternary ammonium salts, as well as nonquaternary amines and amine salts.

Compositions containing cationic nitrogenous compounds in the form of quaternary ammonium salts and substituted imidazolinium salts having two long chain acyclic aliphatic hydrocarbon groups provide fabric softening benefits when used in laundry rinse operations. (See, for example, U.S. Pat. Nos. 3,644,203, Lamberti et al., issued Feb. 22, 1972; and 4,426,299, Verbruggen, issued Jan. 17, 1984; also "Cationic Surface Active Agents as Fabric Softeners," R.R. Egan, Journal of the American Oil Chemists' Society, January 1978, pages 118-121; and "How to Choose Cationics for Fabric Softeners," J.A. Ackerman, Journal of the American Oil Chemists' Society, June 1983, pp. 1166-1169).

Other suitable fabric softening compounds are the nonquaternary amides and the nonquaternary amines. A commonly cited material is the reaction product of higher fatty acids with hydroxy alkyl alkylene diamines. An example of these materials is the reaction product of higher fatty acids and hydroxyethylethylenediamine (See "Condensation Products from beta-hydroxyethylethylenediamine and Fatty Acids or Their Alkyl Esters and Their Application as Textile Softeners in Washing Agents," H.W. Eckert, Fette-Seifen-Anstrichmittel, September 1972, pages 527-533). These materials are usually cited generically along with other cationic quaternary ammonium salts and imidazolinium salts as softening actives in fabric softening compositions. (See U.S. Pat. Nos. 4,460,485, Rapisarda et al., issued July 17, 1984; 4,421,792, Rudy et al., issued Dec. 20, 1983; 4,327,133, Rudy et al., issued April 27, 1982).

A particularly preferred fabric softener is in the form of an aqueous dispersion comprising from 3% to 35% by weight of a mixture consisting of:
(a) from 10% to 92% of the reaction product of a higher fatty acid with a polyamine selected from the group consisting of hydroxyalkylalkylenediamines and dialkylenetriamines and mixtures thereof, and
(b) from 8% to 90% of cationic nitrogenous salts having only one long chain acyclic aliphatic C₁₅-C₂₂ hydrocarbon group, and optionally,
(c) from 0% to 80% of a cationic nitrogenous salt having two or more long chain acyclic aliphatic C₁₅-C₂₂ hydrocarbon groups or one said group and an arylalkyl group having from 15 to 22 carbon atoms in its alkyl chain.
For a detailed description of some preferred fabric softeners, see commonly assigned U.S. Pat. No. 4,661,269, Trinh/Wahl/Swartley/Hemingway, issued Apr. 28, 1987.

The terms herein, e.g., softener compound, in general, denotes both singular and plural unless otherwise specified.

Preferred carriers are liquids selected from the group consisting of water and mixtures of water and short chain C₁-C₄ monohydric alcohols. The water which is used can be distilled, deionized, and/or tap water. Mixtures of water and up to 10%, preferably less than 5%, of short chain alcohol such as ethanol, propanol, isopropanol or butanol, and mixtures thereof, are also useful as the carrier liquid. Carriers which are primarily water are desirable.

Some short chain alcohols are present in commercially available quaternary ammonium compound products. Such products can be used in the preparation of preferred aqueous compositions of the present invention. The short chain alcohols are normally present in such products at a level of from 0.5% to 10% by weight of the aqueous compositions.

### Some Optional Ingredients and Preferred Embodiments

Compatible adjuvants can be added to the compositions herein for their known purposes. Such adjuvants include, but are not limited to, viscosity control agents, perfumes, emulsifiers, preservatives, antioxidants, bactericides, fungicides, colorants, dyes, fluorescent dyes, brighteners, opacifiers, freeze-thaw control agents, soil release agents, and shrinkage control agents, and other agents to provide ease of ironing (e.g., starches). These adjuvants, if used, are added at their usual levels, generally each of up to 5% by weight of the preferred liquid composition.

Viscosity control agents can be organic or inorganic in nature. Examples of organic viscosity modifiers are fatty acids and esters, fatty alcohols, and water-miscible solvents such as short chain alcohols. Examples of inorganic viscosity control agents are water-soluble ionizable salts. A wide variety of ionizable salts can be used. Examples of suitable salts are the halides of the group IA and IIA metals of the Periodic Table of the Elements, e.g., calcium chloride, magnesium chloride, sodium chloride, potassium bromide, and lithium chloride. Calcium chloride is preferred. The ionizable salts are particularly useful during the process of mixing the ingredients to make the liquid compositions herein, and later to obtain the desired viscosity. The amount of ionizable salts used depends on the amount of active ingredients used in such compositions and can be adjusted according to the desires of the formulator. Typical levels of salts used to control the composition viscosity are from 20 to 6,000 parts per million (ppm), preferably from 20 to 4,000 ppm by weight of the composition.

Soil release agents, usually polymers, are desirable additives at levels of from 0.1% to 5%. Suitable soil release agents are disclosed in U.S. Pat. Nos. 4,702,857, Gosselink, issued Oct. 27, 1987; 4,711,730, Gosselink and Diehl, issued Dec. 8, 1987; 4,713,194, Gosselink issued Dec. 15, 1987; and mixtures thereof. Other soil release polymers are disclosed in U.S. Pat. Nos.: 4,749,596, Evans, Huntington, Stewart, Wolf, and Zimmerer, issued June 7, 1988; 3,928,213, Temple, Heuring, and Prentice, issued Dec. 23, 1975; 4,136,038, Pracht and Burns, issued Jan. 23, 1979; and 4,661,267, Dekker, Konig, Straathof, and Gosselink, issued Apr. 28, 1987.

Typical levels of compatible bactericides used in the present compositions are from 1 to 1,500 ppm by weight of the composition.

Examples of antioxidants that can be added to the compositions of this invention are propyl gallate, available from Eastman Chemical Products, Inc., under the trade names Tenox® PG and Tenox S-1, and butylated hydroxy toluene, available from UOP Process Division under the trade name Sustane® BHT.

The compositions can contain other silicone fluids to provide additional benefits such as improved fabric feel. The preferred adjunct silicones are polydimethylsiloxanes of viscosity of from 100 centistokes (cs) to 100,000 cs, preferably from 200 cs to 60,000 cs. These adjunct silicones can be used as is, or can be conveniently added to the softener compositions in a preemulsified form which is obtainable directly from suppliers. Examples of these preemulsified silicones are 60% emulsion of polydimethylsiloxane (350 cs) sold by Dow Corning Corporation under the trade name DOW CORNING® 1157 Fluid and 50% emulsion of polydimethylsiloxane (10,000 cs) sold by General Electric Company under the trade name General Electric® SM 2140 Silicones. The optional silicone component can be used in an amount of from 0.1% to 6% by weight of the composition.

A preferred composition contains from 1 ppm to 1,000 ppm of bactericide, from 0.2% to 2% of perfume, from 0% to 3% of polydimethylsiloxane, from 0% to 0.4% of calcium chloride, from 10 ppm to 100 ppm of dye, and from 0% to 10% of short chain alcohols, by weight of the total composition.

The pH of the preferred compositions of this invention is generally adjusted to be in the range of from 2 to 11, preferably from 2 to 8. Adjustment of pH is normally carried out by including a small quantity of free acid or free base in the formulation. Any acidic material can be used; its selection can be made by anyone skilled in the softener arts on the basis of cost, availability, or safety. Any suitable acid can be used to adjust pH. Preferred are hydrochloric, sulfuric, phosphoric and formic acid. Similarly, any suitable base, e.g., sodium hydroxide, can also be used to adjust pH. For the purposes of this invention, pH is measured by a glass electrode in full strength softening composition in comparison with a standard calomel reference electrode.

The compositions of the present invention can be prepared by a number of methods. Some convenient and satisfactory methods are disclosed in the following nonlimiting examples.

All parts, percentages, and ratios herein are by weight unless otherwise specified.

### EXAMPLE I

### Procedure A

A liquid fabric softener composition containing a micro emulsified amine curable silicone is prepared in the following manner. About 4.33 parts di(hydrogenated tallow)dimethylammonium chloride (DTDMAC), about 1.00 part methyl-1-tallow amidoethyl-2-tallowimidazolinium methylsulfate and about 0.025 parts of a 1% dye solution are weighed into a premix vessel.

After heating to about 75°C and mixing, the premix is added, with agitation, to a mix vessel (44°C) containing about 88.14 parts distilled water and about 0.025 parts antioxidant solution. Then about 0.45 parts of perfume is added to this "main" mix. The main mix is then cooled to about 21°C, to which is added, with stirring, about 7.15 parts amine functional silicone microemulsion (about 14% silicone).

### Procedure B

Same as Procedure A, except that the amine functional silicone microemulsion is incorporated into the main mix prior to cooling of the mix to 21°C.

### EXAMPLE II

A microemulsified amine functional silicone and fabric softener composition is prepared using Procedure A. The approximate levels of the ingredients are: 2.00 parts Mazamide 6, 0.80 parts MTTMAC, 4.03 parts DTDMAC (defined hereinbefore), 1.00 parts of the imidazolinium salt in Example I, 0.42 parts perfume, 1.28 parts alcohol (from actives), 10.00 parts 14% microemulsified amine functional silicone, and the balance is distilled water. See Table 2 and Example I for a recap of the ingredients and method of preparation.

### EXAMPLE III

A microemulsified amine functional silicone and fabric softener composition is prepared using Procedure A. The approximate levels of ingredients are: 17.50 parts Mazamide 6, 6.50 parts DTDMAC, 1.32 parts perfume, 2.07 parts alcohol (from actives), 12.00 parts 14% micro emulsified amine functional silicone, and the balance is distilled water. See Table 2 and Example I for a recap of the ingredients and method of preparation.

### EXAMPLE IV

Intrinsic performance of: Q2-7224 (macroemulsion of Q2-8075, 35% silicone) vs. X2-8406 (microemulsion of Q2-8075, 14% silicone). 9.34 grams of Q2-7224 and 23.35 grams of X2-8406 are used as rinse-added fabric softeners to treat poly-cotton (65%/35%) fabrics (concentration of about 50 ppm in the rinse). The fabrics are treated via one wash (no detergent)/rinse/dry treatment. Shear hysteresis measurements are completed on four fabrics of each treatment. The results below show Q2-7224 to be the better softener system for reducing fiber-fiber and yarn-yarn friction.

| Chart 1 Average Shear Hysteresis (gf/cm) at 2-1/2° and 400g force | |
|---|---|
| X2-8406 | Q2-7224 |
| 1.53 | 1.35 |

Significant at >95% confidence based on a paired t-test calculation.

### EXAMPLE V

### Product C

A microemulsified amine functional silicone and fabric softener composition is prepared using Procedure A. The approximate levels of ingredients are: 3.75 parts DTDMAC, 3.40 parts imidazoline, 0.57 parts MTTMAC, 0.40 parts perfume, 0.025 parts dye, 0.77 parts alcohol (from actives), 0.4-0.9 parts HCl, 7.15 parts MAFS (14%) and the balance is distilled water. This composition contains about 1% amine functional silicone fluid.

### Comparative Product D

A fabric softener composition is prepared as in Product C, except that about 3.03 parts amine functional silicone macroemulsion (33% silicone) is added. This composition contains about 1% amine functional silicone fluid.

See Table 3, for a recap of ingredients for Products C and D. Both Products C and D contain about 1% Q2-8075 amine functional silicone fluid.

Products C & D are used as rinse-added fabric softeners to treat poly cotton (65%/35%) fabrics. The fabrics are treated via one wash/rinse/dry treatment. The detergents used are TIDE® and LIQUID TIDE®. Six sets (DOWNY®, DOWNY plus X2-8406, and DOWNY plus Q2-7224) of swatches saw only TIDE, 6 sets (DOWNY plus X2-8406, and DOWNY plus Q2-7224) of swatches only LIQUID TIDE. Keeping the LIQUID TIDE and TIDE washed fabrics separate, the fabrics were subjected to shear hysteresis measurements. The results below show X2-8406 fabric softener composition to be the better composition for reducing shear hysteresis than the corresponding Q2-8075 composition.

| Chart 2 Average Shear Hysteresis (gf/cm) at 2-1/2° and 400g force | | | |
|---|---|---|---|
| | | DOWNY® + | DOWNY® + |
| | DOWNY® | Q2-7224 | X2-8406 |
| TIDE Wash | 0.69 | 0.71 | 0.65 (a) |
| LIQUID TIDE Wash | 0.88 | 0.78 | 0.76 (b) |
| Average | 0.79 | 0.74 | 0.71 (c) |

| | | | |
|---|---|---|---|
| (a) Significantly lower than DOWNY + Q2-7224 at >95% confidence based on a paired t-test comparison. Significantly lower than DOWNY at >95% confidence based on a paired t-test comparison. | | | |
| (b) Significantly lower than DOWNY + Q2-7224 at ≥70% confidence. Significantly lower than DOWNY at >95% confidence. | | | |
| (c) Significantly lower than DOWNY + Q2-7224 at >95% confidence. Significantly lower than DOWNY at >95% confidence. | | | |

**TABLE 3**

| | Example V | |
|---|---|---|
| | Product C | Product D |
| Ingredient | Approx. Wt.% | Approx. Wt.% |
| MTTMAC¹ | 0.57 | 0.57 |
| DTDMAC² | 3.75 | 3.75 |
| Imidazoline³ | 3.40 | 3.40 |
| Perfume | 0.40 | 0.40 |
| Polar Brilliant Blue Dye Solution | 0.025 | 0.025 |
| Alcohol (from actives) | 0.77 | 0.77 |
| Microemulsified Amine Functional Silicone⁴ (14%) | 7.15 | - |
| Macroemulsified Amine Functional Silicone⁵ | - | 3.03 |
| HCl (31.5%) | 0.4-0.9 | 0.4-0.9 |
| Distilled Water | Balance | Balance |

| | | |
|---|---|---|
| ¹ Mono(hydrogenated tallow)trimethyl ammonium chloride | | |
| ² Di(hydrogenated tallow)dimethyl ammonium chloride | | |
| ³ 1-hydrogenated tallow amidoethyl-2-hydrogenated tallow imidazoline | | |
| ⁴ Dow Corning X2-8406 (described hereinabove) | | |
| ⁵ Dow Corning Q2-7224, a macroemulsion analogue of the microemulsified X2-8406 also containing Dow Corning Q2-8075 silicone fluid. | | |

The incorporation of the microemulsified amine functional silicone delivered via a liquid fabric softener matrix shows improved reduction in shear hysteresis on poly-cotton fabric relative to the traditional macroemulsion delivered via a liquid fabric softener matrix.

## Claims

1. A liquid fabric softening composition comprising:
a)-a microemulsified amino functional silicone of average molecular weight of from 1,000 to 1,000,000,
b)- a fabric softener compound selected from quaternary ammonium compounds, fatty amine compounds, fatty amide compounds, fatty acid compounds, fatty alcohol compounds and mixtures thereof,
c)- a suitable carrier material for a) and b), and
wherein said microemulsified amino functional silicone is obtained by emulsion polymerisation of lower molecular weight polymer selected from silicone polymers, silicone monomers and mixtures thereof, and
wherein said fabric softener compound is in amount from 2% to 35% by weight of the composition.

2. A liquid fabric softening composition according to Claim 1, wherein said microemulsified amino functional silicone is in amount of 0.05% to 25%, preferably from 0.1% to 15% and more preferably from 0.5% to 10% by weight of the composition.

3. A liquid fabric softening composition according to either one of Claim 1 or 2, wherein the weight ratio of said microemulsified amino functional silicone to said fabric softener is from 10:1 to 1:100, preferably from 1:1 to 1:10, more preferably from 1:5 to 1:10.

4. A liquid fabric softening composition according to any one of Claims 1-3, wherein said fabric softener is a quaternary ammonium compound.

5. A liquid fabric softening composition according to any one of Claims 1-3, wherein said fabric softener is a mixture of quaternary ammonium compounds, fatty amine compounds and fatty amide compounds.

6. A liquid fabric softening composition according to any one of Claims 1-3, wherein said fabric softener is a fatty amine compound.

7. A liquid fabric softening composition according to any one of Claims 1-6, wherein said fabric softener is in amount of 4% to 27% by weight of the composition.

8. A method of reducing fiber-fiber/yarn-yarn friction in treated fabrics comprising contacting said fabrics with an effective amount of a liquid fabric softening composition as claimed in any one of Claim 1-7 diluted with water.

## Patentansprüche

1. Flüssige gewebeweichmachende Zusammensetzung, umfassend:
a) ein mikroemulgiertes aminofunktionelles Silikon mit einem mittleren Molekulargewicht von 1.000 bis zu 1.000.000,
b) eine Gewebeweichmacherverbindung, welche unter quaternären Ammoniumverbindungen, Fettaminverbindunqen, Fettamidverbindungen, Fettsäureverbindungen, Fettalkoholverbindungen und Gemischen hievon ausgewählt ist,
c) ein geeignetes Trägermaterial für a) und b), und
wobei das genannte mikroemulgierte aminofunktionelle Silikon durch Emulsionspolymerisation von einem Polymer mit niedrigerem Molekulargewicht erhalten wird, welches Polymer unter Silikonpolymeren, Silikonmonomeren und Gemischen hievon ausgewählt ist, und wobei die genannte Gewebeweichmacherverbindung in einer Menge von 2 Gew.-% bis 35 Gew.-% der Zusammensetzung vorliegt.

2. Flüssige gewebeweichmachende Zusammensetzung nach Anspruch 1, wobei das genannte mikroemulgierte aminofunktionelle Silikon in einer Menge von 0,05 Gew.-% bis 25 Gew.-%, vorzugsweise von 0,1 Gew.-% bis 15 Gew.-% und stärker bevorzugt von 0,5 Gew.-% bis 10 Gew.-% der Zusammensetzung vorliegt.

3. Flüssige gewebeweichmachende Zusammensetzung nach einem der Ansprüche 1 oder 2, wobei das Gewichtsverhältnis von dem genannten mikroemulgierten aminofunktionellen Silikon zu dem genannten Gewebeweichmacher von 10:1 bis 1:100, vorzugsweise von 1:1 bis 1:10, stärker bevorzugt von 1:5 bis 1:10 reicht.

4. Flüssige gewebeweichmachende Zusammensetzung nach einem der Ansprüche 1 bis 3, wobei der genannte Gewebeweichmacher eine quaternäre Ammoniumverbindung ist.

5. Flüssige gewebeweichmachende Zusammensetzung nach einem der Ansprüche 1 bis 3, wobei der genannte Gewebeweichmacher ein Gemisch aus quaternären Ammoniumverbindungen, Fettaminverbindungen und Fettamidverbindungen ist.

6. Flüssige gewebeweichmachende Zusammensetzung nach einem der Ansprüche 1 bis 3, wobei der genannte Gewebeweichmacher eine Fettaminverbindung ist.

7. Flüssige gewebeweichmachende Zusammensetzung nach einem der Ansprüche 1 bis 6, wobei der genannte Gewebeweichmacher in einer Menge von 4 Gew.-% bis 27 Gew.-% der Zusammensetzung vorliegt.

8. Verfahren zur Verringerung der Faser-Faser/Garn-Garn-Reibung in behandelten Geweben, umfassend das In-Kontakt-Bringen der genannten Gewebe mit einer mit Wasser verdünnten wirksamen Menge einer flüssigen gewebeweichmachenden Zusammensetzung, wie sie in einem der Ansprüche 1 bis 7 beansprucht ist.

## Revendications

1. Composition liquide d'assouplissant textile comprenant:
a) une silicone amino-fonctionnelle microémulsifiée de masse moléculaire moyenne 1 000 à 1 000 000,
b) un composé assouplissant textile choisi parmi les composés d'ammonium quaternaire, les composés d'amines grasses, les composés d'amides gras, les composés d'acides gras, les composés d'alcools gras, et leurs mélanges,
c) un véhicule convenable pour a) et b), et
dans laquelle ladite silicone amino-fonctionnelle microémulsifiée est obtenue par polymérisation en émulsion d'un polymère de masse moléculaire plus faible choisi parmi les polymères silicones, les monomères silicones et leurs mélanges, et
dans laquelle ledit composé assouplissant textile est présent à raison de 2% à 35% en poids de la composition.

2. Composition liquide d'assouplissant textile selon la revendication 1, dans laquelle ladite silicone amino-fonctionnelle microémulsifiée est présente à raison de 0,05% à 25%, de préférence de 0,1% à 15% et mieux encore de 0,5% à 10%, en poids de la composition.

3. Composition liquide d'assouplissant textile selon l'une quelconque des revendications 1 ou 2, dans laquelle le rapport pondéral de ladite silicone amino-fonctionnelle microémulsifiée audit assouplissant textile est de 10:1 à 1:100, de préférence de 1:1 à 1:10, mieux encore de 1:5 à 1:10.

4. Composition liquide d'assouplissant textile selon l'une quelconque des revendications 1-3, dans laquelle ledit assouplissant textile est un composé d'ammonium quaternaire.

5. Composition liquide d'assouplissant textile selon l'une quelconque des revendications 1-3, dans laquelle ledit assouplissant textile est un mélange de composés d'ammonium quaternaire, de composés d'amines grasses et de composés d'amides gras.

6. Composition liquide d'assouplissant textile selon l'une quelconque des revendications 1-3, dans laquelle ledit assouplissant textile est un composé d'amine grasse.

7. Composition liquide d'assouplissant textile selon l'une quelconque des revendications 1-6, dans laquelle ledit assouplissant textile est présent à raison de 4% à 27% en poids de la composition.

8. Procédé de réduction du frottement fibre à fibre ou fil à fil dans des tissus traités, comprenant la mise en contact desdits tissus avec une quantité efficace d'une composition liquide d'assouplissant textile selon l'une quelconque des revendications 1-7, diluée avec de l'eau.
